

## UNITED STATES PATENT OFFICE

1,985,783

## METHOD OF MANUFACTURING LAMINATED METAL BANDS

Franz Jordan, Berlin-Charlottenburg, Germany

No Drawing. Application December 23, 1932,  
Serial No. 648,645. In Germany November 6,  
1932

## 4 Claims. (Cl. 29—189)

The quality of the projection of cinematographic pictures by reflected light instead of by light passing directly through a translucent film depends not only upon the clearness of the pictures and the strength of the light, but also on the reflecting surface employed.

It has been found by experiment that aluminium, on account of its white metallic lustre, is excellent as a reflecting surface. This appears 10 all the more favorable inasmuch as the light weight of aluminium brings it clearer to the usual very light cellulose film. Nevertheless, it has been already found that a film strip of aluminium as light in weight as a cellulose film 15 and correspondingly thinner than the latter does not stand up well in use. It has, therefore, been proposed to use a steel strip or band having an aluminium coating instead of a cellulose film. Every form of aluminium coating or covering is, 20 however, not suitable for the purpose, due to optical requirements.

Now, according to the present invention, for the purpose of applying the aluminium coating or covering so that it will have the brightest lustre 25 and light-reflecting power and be free from spots and blemishes, a magnetic iron core is taken and also an aluminium covering for each side thereof, and the whole passed in heated state through between pressure rollers which are smooth, clean 30 and have a lustrous polish, the pressure of the core and its coverings continuing until a film band thinness approximately from 0.03 to 0.05 of a millimeter is attained.

It has been found that by alloying aluminium 35 with precious metals, for example silver, the lustre and light-reflecting power of the aluminium covering is increased, and as a further feature of my invention such an alloy may be employed to form the coverings for the iron core referred to.

With the small thickness of the aluminium iron-cored film band, about from 0.03 to 0.05 of a millimeter, the coverings themselves must, of course, be correspondingly thin, some thousandths of a millimeter. As the plating and rolling process from the thicker iron and coverings 40 proceeds towards attainment of the final desired thinness, it is necessary, to achieve on the film band a surface free from objections, that the whole plating and rolling out process be undertaken with rollers having a high and lustrous 45 polish, their surfaces being free of ripples or rough places, as the aluminium covering, as also a covering of aluminium and silver is weak and impressionable. Further, a coating or covering 50 must be rolled upon both sides of the iron core

of the band, the latter being, thus, non-inflammable and rustless. These precautions being observed, there is no difficulty in rolling out the aluminium coverings to the thickness above mentioned, as the aluminium by the roller process is smoothly applied and slipping between the rollers is prevented. The rolling pressure can be higher than with iron alone, as the latter at high pressure easily slips and tears. The band, as a whole, is lowered in weight as a result of its 10 covering with the aluminium so that its excess of weight over the other bands, such as those of celluloid and other materials, is only trifling.

Further, the band according to this invention has strong magnetic properties so that it is very 15 suitable for use with magnetic tone films. Both the picture and the sound in a tone film can, therefore, be photographed together, exactly as in celluloid films. Still further, the band of this invention is valuable for the projection of colored films, as through the indirect projection over the metallic covering of the band the colors 20 appear clear and unaltered. This is never the case with even a fully clear film band through which light is projected, as in such conditions 25 the colors do not come out exactly true upon the screen. It will be understood that the metal band may have printed thereon in black or in colors any notices or textual additions, and these 30 may be projectable.

Not only does the band made according to this invention show all advantages possessed by hitherto proposed film bands, but it adds the advantage that it is fireproof and will not alter when 35 kept in store which is not the case with known celluloid film bands. The new band is also weldable; this increases its utility as a plurality of such bands may be electrically welded together 40 at their ends. The cost of production is lower than that of most known forms of film bands.

I claim:

1. A mode of carrying out the method for manufacturing laminated metal bands suited as carriers for speaking films and comprising unwinding from individual spools an iron band serving as core in the laminated band to be made, and two aluminium bands serving as coverings for said core, heating the three bands, and uniting them with one another by welding them together in hot state between pressing rollers, said mode comprising employing for the coverings an alloy of aluminium and a small addition of a precious metal having a white lustre, and transforming the laminated band into foils of a thickness of 55

from 0.03 to 0.05 mm between polished rollers of a polishing mill.

2. A mode of carrying out the method for manufacturing laminated metal bands suited as carriers for speaking films and comprising, unwinding from individual spools an iron band serving as core in the laminated band to be made, and two aluminium bands serving as coverings for said core, heating the three bands and uniting them with one another by welding them together in hot state between pressing rollers, said mode comprising employing for the coverings an alloy of aluminium and a small addition of silver; and transforming the laminated band into foils of a thickness of from 0.03 to 0.05 mm between polished rollers of a polishing mill.
3. A mode of carrying out the method for manufacturing laminated metal bands suited as carriers for speaking films and comprising, unwinding from individual spools an iron band serving as core in the laminated band to be made, and two aluminium bands serving as coverings for

said core, heating the three bands and uniting them with one another by welding them together in hot state between pressing rollers, said mode comprising employing for the coverings an alloy of aluminium and a small addition of silver; and transforming the laminated band into foils of a thickness of from 0.03 to 0.05 mm between polished rollers of a polishing mill.

4. A mode of carrying out the method for manufacturing laminated metal bands suited as carriers for speaking films and comprising, unwinding from individual spools an iron band serving as core in the laminated band to be made, and two aluminium bands serving as coverings for said core, heating the three bands, and uniting them with one another by welding them together in hot state between pressing rollers, said mode comprising employing for the coverings an alloy of aluminium and a small addition of a precious metal having a white lustre and being adapted to prevent the color of the aluminium from changing as otherwise caused by the diffusion between the aluminium and the iron in hot state; and transforming the laminated band into foils of a thickness of from 0.03 to 0.05 mm between highly polished rollers of a polishing mill.
5. A mode of carrying out the method for manufacturing laminated metal bands suited as carriers for speaking films and comprising, unwinding from individual spools an iron band serving as core in the laminated band to be made, and two aluminium bands serving as coverings for

5

10

15

20

25

FRANZ JORDAN.